



US008172641B2

(12) **United States Patent**  
**Ho et al.**

(10) **Patent No.:** **US 8,172,641 B2**  
(b4) **Date of Patent:** **May 8, 2012**

(54) **CMP BY CONTROLLING POLISH TEMPERATURE**

(75) Inventors: **Ming-Che Ho**, Tainan (TW); **Jean Wang**, Hsin-Chu (TW); **Lawrence Chiang Sheu**, Hsin-Chu (TW)

(73) Assignee: **Taiwan Semiconductor Manufacturing Co., Ltd.**, Hsin-Chu (TW)

(\*) Notice: Subject to any disclaimer, the term of this patent is extended or adjusted under 35 U.S.C. 154(b) by 962 days.

(21) Appl. No.: **12/174,762**

(22) Filed: **Jul. 17, 2008**

(65) **Prior Publication Data**

US 2010/0015894 A1 Jan. 21, 2010

(51) **Int. Cl.**  
**B24B 1/00** (2006.01)

(52) **U.S. Cl.** ..... **451/7**; **451/41**; **451/53**  
(58) **Field of Classification Search** ..... **451/7, 41, 451/56, 54, 57, 53**

See application file for complete search history.

(56) **References Cited**

U.S. PATENT DOCUMENTS

3,671,313 A \* 6/1972 Reynolds ..... 38/95  
5,300,155 A 4/1994 Sandhu et al.

5,755,614 A \* 5/1998 Adams et al. ..... 451/60  
5,873,769 A \* 2/1999 Chiou et al. ..... 451/7  
6,099,662 A \* 8/2000 Wang et al. ..... 134/26  
6,264,789 B1 7/2001 Pandey et al. .....  
6,273,099 B1 \* 8/2001 Chang et al. ..... 134/1.3  
6,295,998 B1 \* 10/2001 Kudelka et al. ..... 134/1.3  
6,325,698 B1 \* 12/2001 Wada et al. ..... 451/8  
6,361,407 B1 \* 3/2002 Lu et al. ..... 451/41  
6,409,582 B1 \* 6/2002 Togawa et al. ..... 451/67  
6,749,484 B2 6/2004 Yang et al. .....  
7,883,393 B2 \* 2/2011 Kordic et al. ..... 451/7  
2004/0092210 A1 \* 5/2004 Chen et al. ..... 451/37  
2007/0298692 A1 \* 12/2007 Mavliev et al. ..... 451/56  
2008/0314870 A1 \* 12/2008 Inoue et al. ..... 216/38

FOREIGN PATENT DOCUMENTS

EP 1175964 A2 1/2002

\* cited by examiner

Primary Examiner — Maurina Rachuba

(74) Attorney, Agent, or Firm — Slater & Matsil, L.L.P.

(57) **ABSTRACT**

A method for manufacturing integrated circuits on a wafer includes providing a facility-supplied room temperature solution; controlling the temperature of the facility-supplied room temperature solution to a desired temperature set point to generate a rinse solution; and rinsing a polishing pad using the rinse solution. The wafer is then polished by means of a chemical mechanical polishing process.

**13 Claims, 6 Drawing Sheets**





Fig. 1



Fig. 2



Fig. 3



Fig. 4



Fig. 5



Fig. 6  
Sampling Position

## CMP BY CONTROLLING POLISH TEMPERATURE

### TECHNICAL FIELD

This invention relates generally to integrated circuit manufacturing processes, and more particularly to equipment and methods for carrying out a chemical mechanical polishing (CMP) process.

### BACKGROUND

CMP processes are widely used in the fabrication of integrated circuits. As an integrated circuit is built up layer by layer on the surface of a semiconductor wafer, CMP is used to planarize the topmost layer or layers to provide a level surface for subsequent fabrication steps. CMP is carried out by placing the wafer in a carrier that presses the wafer surface to be polished against a polishing pad attached to a platen disk. Both the platen disk and the wafer carrier are rotated while a slurry containing both abrasive particles and reactive chemicals is applied to the polishing pad. The slurry is transported to the wafer surface via the rotation of the porous polishing pad. The relative movement of the polishing pad and wafer surface coupled with the reactive chemicals in the slurry allows CMP to level the wafer surface by means of both physical and chemical forces.

CMP can be used at a number of points during the fabrication of an integrated circuit. For example, CMP may be used to planarize the inter-level dielectric layers that separate the various circuit layers in an integrated circuit. CMP is also commonly used in the formation of the copper lines that interconnect components of an integrated circuit.

Conventional CMP processes suffer from various drawbacks. First, uniformity, including within-wafer uniformity and wafer-to-wafer uniformity, can be difficult to control. For example, when planarizing a copper interconnect layer, the total (wafer-to-wafer plus within-wafer) variation of the sheet resistance (Rs) of the copper can be more than 15 percent even when the polishing time is adjusted using advanced process controls. Second, conventional CMP processes often fail to remove the desired amount of material from a wafer, which means the wafer needs to be reworked. Conventionally, more than 20 percent of the wafers need to be reworked. Third, many dummy wafers, typically more than 20 dummy wafers per day, may be needed for the conditioning of new polishing pads, and for the conditioning of polishing pads between lots (between which the CMP equipment is idled). Fourth, due to the significant wafer-to-wafer non-uniformity, the lifetimes of the polishing pads can vary significantly from pad to pad. All the above-discussed drawbacks mean that CMP processes can have low producibility and high cost of consumables (such as dummy wafers, polishing pads, and the like).

To solve the above-discussed problems, methods for improving CMP processes have been explored. For example, approaches involving controlling the temperature of the platen disk, wafer carrier, and slurry have been proposed. However, these methods were found to have limited results. New methods with improved results are thus needed.

### SUMMARY OF THE INVENTION

Embodiments of the invention comprise methods for preparing a polishing pad for a CMP process in which a polishing pad is rinsed with a temperature-controlled rinse solution before the pad is used to polish a wafer. The temperature of the rinse solution dispensed onto the wafer differs from room

temperature. The rinse solution may comprise de-ionized (DI) water, or may simply consist of DI water. Furthermore, after the wafer is polished, the polishing pad may be rinsed with a different temperature rinse solution before the next polishing step is carried out.

Other embodiments of the invention include an apparatus for manufacturing integrated circuits, wherein the apparatus includes a polishing pad; a rinse arm configured to be movable over the polishing pad; a pipe connected to the rinse arm; and a temperature controller connected to the pipe. The temperature controller controls the temperature of the rinse solution to a desired temperature set point before the rinse solution is dispensed onto the polishing pad.

The advantageous features of the present invention include improved wafer-to-wafer and within-wafer uniformity, prolonged life of polishing pads, and reduced use of dummy wafers.

### BRIEF DESCRIPTION OF THE DRAWINGS

For a more complete understanding of the present invention, and the advantages thereof, reference is now made to the following descriptions taken in conjunction with the accompanying drawings, in which:

FIG. 1 illustrates a first embodiment of the present invention, a CMP system with a temperature controller employing a tank containing a heat exchange medium;

FIG. 2 illustrates a second embodiment of the present invention, wherein a CMP system with a temperature controller including heat exchange pipes is included in a CMP system;

FIG. 3 illustrates a third embodiment of the present invention, wherein two temperature controllers are included in a CMP system;

FIG. 4 illustrates an integrated circuit structure, on which two successive CMP processes may be effectively employed;

FIG. 5 illustrates the variation in the amount of TaN removed across the diameters of several wafers after the polishing pad used to polish those wafers was rinsed with room temperature de-ionized water; and

FIG. 6 illustrates the variation in the amount of TaN removed across the diameters of several wafers after the polishing pad used to polish those wafers was rinsed with temperature-controlled de-ionized water.

### DETAILED DESCRIPTION OF ILLUSTRATIVE EMBODIMENTS

The making and using of the presently preferred embodiments are discussed in detail below. It should be appreciated, however, that the present invention provides many applicable inventive concepts that can be embodied in a wide variety of specific contexts. The specific embodiments discussed are merely illustrative of specific ways to make and use the invention, and do not limit the scope of the invention.

Exemplary embodiments of the present invention are discussed with reference to FIGS. 1 through 3, which illustrate exemplary CMP systems for performing methods in accordance with the invention. The CMP system in FIG. 1 comprises wafer 16 retained by carrier 10, polishing pad 12 retained on platen disk 13, slurry dispensing nozzle 14, and high-pressure rinse arm 20. Carrier 10 presses the surface of wafer 16 to be polished against polishing pad 12. During the polishing process, polishing pad 12 and wafer 16 are each rotated, and in some embodiments wafer 16 may also be moved along the radius of polishing pad 12. Wafer 16 and polishing pad 12 may be rotated in the same direction, or they

may be counter-rotated in opposite directions. High-pressure rinse arm 20 is used to dispense a rinse solution such as di-ionized (DI) water. High-pressure rinse arm 20 may be moved over polishing pad 12 during the rinse steps, and moved away when no rinse is being performed.

Through pipe 21, high-pressure rinse arm 20 is connected to temperature controller 22. In an embodiment of the present invention, temperature controller 22 is used to ensure that the temperature of the rinse solution dispensed by high-pressure rinse arm 20 is at a desired temperature. The rinse solution may be DI water, although the rinse solution may further comprise small amounts of additives. Accordingly, temperature controller 22 includes inlet 26 for introducing the facility-supplied solution, which is typically at room temperature. Pump 28 may be connected to inlet 26 of temperature controller 22 to control the flow rate of the facility-supplied room temperature solution.

In the embodiment of FIG. 1, temperature controller 22 includes a tank 30 for retaining a volume of heat exchange medium 32. Heat exchange medium 32 may be water, oil, or the like. Embedded elements 34, which may be heating elements or cooling elements, are immersed in heat exchange medium 32, and are used for adjusting the temperature of heat exchange medium 32. Mixer 36 is used to stir heat exchange medium 32 to achieve a substantially uniform temperature in heat exchange medium 32 contained in tank 30. The facility-supplied room temperature solution flows through heat exchange tube 40, which is immersed in heat exchange medium 32. Heat exchange tube 40 can be coiled in order to increase the heat exchange efficiency. Various temperature sensors 44 may be immersed in heat exchange medium 32 to sense its temperature. Temperature sensors 44 may also be connected to pipe 21 to sense the temperature of the rinse solution outputted by temperature controller 22, which will be at a different temperature than the facility-supplied room temperature solution. Thermal insulation 42 may be wrapped around tank 30 and/or pipe 21 to reduce heat loss.

Although referred to as being at room temperature, the facility-supplied solution flowing into inlet 26 may have a higher or lower temperature than the room temperature of the environment, in which the CMP system is located, which temperature may be, for example, between about 20° C. and about 25° C., or about 24° C. After flowing through temperature controller 22, the temperature of the facility-supplied room temperature solution is increased or lowered, for example, by greater than about 2° C., or even greater than about 3° C. Throughout the description, the facility-supplied room temperature solution flowing out of temperature controller 22 is referred to as a rinse solution.

To better effectuate the temperature control of the rinse solution, the CMP system may further include control unit 46. The temperature sensed by temperature sensors 44 may be fed back to control unit 46, which monitors the sensed temperatures, and compares the sensed temperatures with predetermined set points. If the sensed temperatures deviate from the set points, control unit 46 controls embedded elements 34 to adjust the temperature until the temperature of the rinse solution sprayed by high-pressure rinse arm 20 is at the desired temperature.

The temperature-controlled rinse solution may be used in various steps in the CMP. An exemplary CMP process that can be performed by the apparatus shown in FIG. 1 comprises several steps. First, wafer 16 is mounted on carrier 10. A high-pressure rinse with the temperature-controlled rinse solution is then performed by positioning high-pressure rinse arm 20 over polishing pad 12 and spraying the rinse solution onto the rotating polishing pad 12. In the meantime, carrier 10

may be positioned so that wafer 16 stays above polishing pad 12, and hence wafer 16 is not rinsed. Alternatively, wafer 16 may be lowered to contact polishing pad 12, or at least be close enough to polishing pad 12, so that both polishing pad 12 and wafer 16 are rinsed. After the high pressure rinse is complete, high-pressure rinse arm 20 can be moved away from above polishing pad 12.

Next, the slurry is pre-flowed in the slurry dispensing nozzle 14, and in the upstream pipes (not shown) of the slurry dispensing system (not shown) to discard residual slurry and to stabilize the slurry flow rate. Wafer 16 is then polished by simultaneously having carrier 10 press wafer 16 against polishing pad 12, dispensing slurry onto polishing pad 12, and rotating wafer 16 and polishing pad 12. The temperature of the slurry may be controlled independently from the temperature of the rinse solution. Optionally, the temperature of platen disk 13 may be modified by, for example, circulating a liquid coolant within the platen.

After the previous polishing step, a cleaning polish is performed, in which wafer 16 remains in contact with polishing pad 12, and both wafer and pad continue to rotate. During the cleaning polish, high-pressure rinse arm 20 is once again positioned over polishing pad 12, where it once again sprays rinse solution onto polishing pad 12. Since wafer 16 is still in contact with polishing pad 12, wafer 16 is also rinsed. The slurry and the substances generated by the main polish are thus removed, and polishing pad 12 and wafer 16 are cleaned.

During the cleaning polish, instead of using a rinse solution that has its temperature controlled to be either above or below room temperature, a facility-supplied room temperature solution may be used to rinse polishing pad 12 and wafer 16, wherein the facility-supplied room temperature solution may have a temperature substantially close to the room temperature in which the CMP system is located, for example, between about 20° C. and about 25° C., or about 24° C.

After the cleaning polish, wafer 16 is detached from carrier 10, and is subjected to a post-polishing cleaning step. Polishing pad 12 is then rinsed using the temperature-controlled rinse solution. All of the above-discussed CMP process steps may then be performed to polish a subsequent wafer.

In many embodiments the rinse solution has its temperature controlled to be above room temperature. In general, the rinse solution will have a temperature of at least about 2° C. higher than that of the facility-supplied room temperature solution. More preferably, the rinse solution has a temperature between about 26° C. and about 100° C., and even more preferably between about 30° C. and about 65° C. The optimum choice of rinse solution temperature for a given polishing process depends on the material(s) to be removed during the polishing process, the size of the features on the wafer, the features of the pad, and the contents of the slurry. For example, when a bulk copper layer is being polished, the optimum rinse solution temperature is typically between about 30° C. and about 40° C. Alternatively, when a TaN barrier layer is being polished, the optimum rinse solution temperature is between about 40° C. and about 50° C. Since a TaN barrier layer is more patterned than a bulk copper layer, the feature sizes in the pattern of the TaN layer may influence the optimum rinse temperature. In an exemplary embodiment, wafers with smaller nominal feature sizes may be rinsed with rinse solutions having higher temperatures. For example, for a wafer with a nominal feature size of 65 nm the optimum rinse solution temperature may be closer to 40° C., while for wafers with smaller nominal feature sizes of 32 nm or 45 nm the optimum rinse solution temperature may be closer to 50° C.

The increase in the temperature of the rinse solution may be achieved using the embodiment illustrated in FIG. 1, or the alternative embodiments in FIGS. 2 and 3. Advantageously, the heated rinse solution helps promote the chemical reactions of the CMP process. The heated rinse solution will also soften polishing pad 12, which results in better contact between polishing pad 12 and wafer 16. As a result, the mechanical part of the CMP is also improved. Use of embodiments of the present invention can eliminate the need to condition polishing pad 12 by polishing dummy wafers. To be specific, both the first polish performed using a new polishing pad 12 and the first polish after the CMP system has been idled for a while don't have to be performed on dummy wafers. Instead, the above-mentioned first polishes may be performed on actual production wafers having integrated circuits.

In alternative embodiments, the rinse solution has its temperature controlled to be below room temperature. In alternative embodiments, the rinse solution has a temperature lower than that of the facility-supplied room temperature solution with a temperature difference of about 2° C. or greater. More preferably, the rinse solution has a temperature between about 1° C. and about 22° C., and more preferably between about 17° C. and about 22° C. The decrease in the temperature of the rinse solution is achieved using the embodiments illustrated in FIGS. 1 through 3 in which cooler(s) are employed. Experiments have revealed that the reduction in the temperature of the rinse solution results in a reduction in the overall temperature on polishing pad 12. Such reduction in temperature improves the uniformity for polishing certain features, particularly for the polish of bulk copper, wherein the wafer center-edge uniformity can be improved.

FIG. 2 illustrates an alternative CMP system, which uses heat exchange pipes 50 to either heat or cool the facility-supplied room temperature solution. Like reference numerals are used to designate like elements in FIGS. 1 and 2. Heat exchange pipes 50 heat or cool the facility-supplied room temperature solution, and hence the resulting rinse solution may have an increased or decreased temperature compared to that of the facility-supplied room temperature solution flowing into inlet 26. Again, control unit 46 is used to maintain the temperature of the rinse solution dispensed out of high-pressure rinse arm 20 in a desirable range.

The embodiment shown in FIG. 3 comprises a CMP system with two temperature controllers. The system in FIG. 3 may have one temperature controller configured to heat the facility-supplied room temperature solution, and the other configured to cool the facility-supplied room temperature solution. In other embodiments, both temperature controllers may output heated rinse solutions having temperatures different from each other. In yet other embodiments, both temperature controllers may output cooled rinse solutions having temperatures different from each other. In FIG. 3, the CMP system comprises two temperature controllers 22A and 22B, and two high-pressure rinse arms 20A and 20B. Accordingly, both heated and cooled rinse solutions may be provided in a single CMP system, which may be used for polishing different features on a single wafer or on different wafers, as will be discussed in subsequent paragraphs.

The CMP system shown in FIG. 3 may be used to achieve optimum results for combinations of CMP processes. FIG. 4 illustrates a damascene structure on which two CMP processes are performed. The damascene structure includes low-k dielectric layer 60, (diffusion) barrier layer 62, and bulk copper 64. Diffusion barrier layer 62 may be formed of titanium, titanium nitride, tantalum, tantalum nitride, or the like. A first CMP process is performed to remove the bulk copper 64 until diffusion barrier layer 62 is exposed. The first CMP

may stop at dotted line 66. A second CMP process is then performed to remove the exposed diffusion barrier layer 62 until low-k dielectric layer 60 is exposed. In an embodiment, the first CMP process, which removes bulk copper 64, is performed after polishing pad 12 is rinsed with a cooled rinse solution, for example, with a temperature of about 20° C. and about 22° C. Alternatively, the first CMP process may be performed after polishing pad 12 is rinsed with a rinse solution heated to between about 30° C. to about 40° C. Either one of the heated or cooled rinses will improve the uniformity of the first CMP process. The second CMP process, which removes diffusion barrier layer 62, is performed with polishing pad 12 rinsed with a heated rinse solution, for example when the barrier layer is TaN, with a temperature of about 40° C. to about 50° C. By employing two different temperature rinses, the uniformity of each of the two CMP processes can be optimized.

The embodiments of the present invention have significantly improved the CMP processes. To compare the results of the embodiments of the present invention and the results of prior art embodiments, two groups of samples were made, with the first group of sample wafers rinsed by room temperature DI water before the respective main polishes, and the second group of sample wafers rinsed by 50° C. DI water before the respective main polishes. The CMP processes were carried out on an Applied Materials Reflexion LK CMP system using a JTS 009-5 polishing pad and JSR T3B slurry. The flow rate of the rinse solutions (either room temperature or temperature controlled) was 8 L/min. Experimental results revealed that over a period of half a month, the monitored standard deviation of removal rates was reduced from a relative value of 56.53 for the first group of samples to a relative value of 34.46 for the second group of sample wafers. The non-uniformity mean was reduced from 7.83 percent for the first group of samples to 4.35 percent for the second group of sample wafers. The center-to-edge difference mean was reduced from 29.30 Å for the first group of sample wafers to 11.01 Å for the second group of sample wafers. Further experiments revealed that over the lifetime of a polishing pad, which was used to polish 580 wafers, the thicknesses of the polished features were always within the target, even though no adjustment of polishing time was performed, no dummy wafer polishes were performed, and no rework was performed.

FIGS. 5 and 6 compare the material removal rate profiles for a CMP process employing a room temperature rinse (FIG. 5) and a CMP process employing a temperature-controlled rinse (FIG. 6). The previously described CMP system, polishing pad, and slurry were used to generate the results shown in FIGS. 5 and 6. The graphs in FIGS. 5 and 6 show the removal rate profiles for CMP processes in which the material being removed is a TaN barrier. In those graphs, the Y-axis indicates the amount of material removed in Å, while the points along the X-axis correspond to locations along a diameter of a wafer, with point 25 being the center of the wafer, and points 1 and 49 being the opposite edge points of the wafer. In each of FIGS. 5 and 6, the lower lines (for example, lines 70 and 80) show the results obtained when the respective polishing pads have been used to polish a relatively smaller number of wafers, while the higher lines (for example, lines 76 and 88) show the results obtained after the respective polishing pads have been used to polish a relatively greater number of wafers.

Referring to FIG. 5, whose sample wafers were rinsed with room temperature DI water, it is found that when the respective polishing pad was used to polish a smaller number of wafers (for example, 100 pieces for line 70), the center por-

tion of the respective wafer has a lower removal rate of TaN than the edge portions of the wafer. After more wafers are polished using the same polishing pad, the removal rate of TaN at the center of the wafer increases, and eventually, the center portion has a greater removal rate than the edge portions. As a comparison, FIG. 6 shows the results obtained from sample wafers rinsed using 50° C. DI water. It is found that throughout the lifetime of the polishing pad, the center removal rate of TaN is always close to the edge removal rate. Furthermore, the removal rate profile remains unchanged as the number of wafers processed by the polishing pad increases.

The embodiments of the present invention have several advantageous features. First, the uniformities (including within-wafer uniformity and wafer-to-wafer uniformity) of the polish processes are significantly improved. That improvement can significantly reduce or even eliminate the need to rework wafers or to adjust the polishing time by monitoring the removal rate with dummy wafers. The amount of needed CMP consumables is significantly reduced due to the substantial elimination of dummy wafer polishes, prolonged life of polishing pads, and the reduction in reworking.

Although the present invention and its advantages have been described in detail, it should be understood that various changes, substitutions and alterations can be made herein without departing from the spirit and scope of the invention as defined by the appended claims. Moreover, the scope of the present application is not intended to be limited to the particular embodiments of the process, machine, manufacture, and composition of matter, means, methods and steps described in the specification. As one of ordinary skill in the art will readily appreciate from the disclosure of the present invention, processes, machines, manufacture, compositions of matter, means, methods, or steps, presently existing or later to be developed, that perform substantially the same function or achieve substantially the same result as the corresponding embodiments described herein may be utilized according to the present invention. Accordingly, the appended claims are intended to include within their scope such processes, machines, manufacture, compositions of matter, means, methods, or steps.

What is claimed is:

1. A method for preparing a polishing pad for a chemical mechanical polishing (CMP) process, the method comprising:

cooling a first rinse solution to a first desired temperature set point;

rinsing the polishing pad with the first rinse solution at the first desired temperature set point; and after the rinsing step, subjecting a surface of a first wafer to the CMP process.

5 2. The method of claim 1, wherein the temperature-controlled first rinse solution is de-ionized water.

3. The method of claim 1, wherein the first desired temperature set point differs from a room temperature of an environment in which the CMP process is being carried out 10 by more than about two degrees centigrade, and wherein the room temperature is between about 20° C. and about 25° C.

4. The method of claim 1, wherein the step of cooling the first rinse solution is performed using heat exchange pipes.

5. The method of claim 1, wherein the first desired temperature set point is between about 1° C. and about 22° C.

15 6. The method of claim 1, wherein the step of cooling the first rinse solution is performed by a temperature controller comprising a heat exchange medium.

7. The method of claim 1 further comprising, after the step 20 of subjecting the surface of the first wafer to the CMP process, rinsing the polishing pad with a room temperature rinse solution at a temperature between about 20° C. and about 25° C.

8. The method of claim 1 further comprising, after the step 25 of subjecting the surface of the first wafer to the CMP process, rinsing both the polishing pad and the first wafer with a room temperature rinse solution at a temperature between about 20° C. and about 25° C.

9. The method of claim 1 further comprising:  
heating the temperature of a second rinse solution to a 30 second desired temperature set point;  
rinsing the polishing pad with the second rinse solution;  
and  
after the rinsing step using the second rinse solution, subjecting a surface of a second wafer to an additional CMP 35 process.

10. The method of claim 9, wherein the first wafer is the same as the second wafer.

11. The method of claim 9, wherein the surface of the first wafer comprises copper and the first desired temperature set 40 point is between about 20° C. and about 22° C., and the second desired temperature set point is between about 40° C. and about 50° C.

12. The method of claim 1, wherein the surface of the first wafer comprises copper.

45 13. The method of claim 9, wherein the surface of the second wafer comprises TaN.

\* \* \* \* \*